

R. R. ROSENBAUM.  
MANUFACTURE OF ASPHALT.  
APPLICATION FILED APR. 2, 1915. RENEWED JULY 29, 1918.  
**1,332,359.**

Patented Mar. 2, 1920.



Inventor:

Rudolph R. Rosenbaum

By Gillam & Gillam, Attys.

# UNITED STATES PATENT OFFICE.

RUDOLPH R. ROSENBAUM, OF CHICAGO, ILLINOIS, ASSIGNOR TO CENTRAL COMMERCIAL COMPANY, OF CHICAGO, ILLINOIS, A CORPORATION OF ILLINOIS.

## MANUFACTURE OF ASPHALT.

1,332,359.

Specification of Letters Patent.

Patented Mar. 2, 1920.

Application filed April 2, 1915, Serial No. 18,857. Renewed July 29, 1918. Serial No. 247,314.

To all whom it may concern:

Be it known that I, RUDOLPH R. ROSENBAUM, a subject of the Emperor of Germany, and resident of Chicago, county of Cook, and 5 State of Illinois, have invented certain new and useful Improvements in the Manufacture of Asphalt, of which the following is a specification.

The invention relates to a process of treating solid mineral bitumens for producing materials of improved quality and having a wider range of commercial utility and to asphalt which may be produced by the said process. Some of the solid mineral bitumens, more particularly the asphaltites, or so-called asphaltic coals, are wholly non-melted while others are only imperfectly meltable. That is to say, the minerals referred to are subject either to a complete or 20 to a partial destructive distillation by heat before a melting temperature is reached.

A mineral of the kind described occurs in considerable quantity at Sardis, near Tuskanoma, Pushmataha county, Oklahoma, and 25 is now commercially known as grahamite. This mineral is obtainable substantially free from earthy substances. Some samples are soluble to the extent of ninety-seven per cent. of their weight in carbon bisulfid and contain scarcely one per cent. of inorganic mineral matter. In its original condition, however, the mineral is a black, hard, but friable substance, scarcely distinguishable in appearance from anthracite coal. On being 30 heated it decomposes without the slightest evidence of melting, and is readily inflammable. Similar asphaltites occur in other localities, for example, albertite.

The non-melted or imperfectly meltable 40 character of these asphaltites renders them quite unfit in their natural state for many of the commercial uses to which the meltable solid bitumens have been applied. The present invention accordingly contemplates a process by which the non-melted and imperfectly meltable asphaltites are transformed into perfectly meltable products having increased commercial value and the said products. The object of the invention is to 45 provide a simple and inexpensive process for accomplishing this result.

In the accompanying drawings—

Figure 1 is a central sectional view partly in elevation, showing a form of apparatus

in which the improved process may be carried out, and

Figs. 2 and 3 are transverse sectional views taken on the lines 2—2 and 3—3 respectively, of Fig. 1.

The meltable asphalts, as, for example, natural uintahite (gilsonite), are perfectly soluble in carbon tetrachlorid and are frequently regarded as consisting of a mixture of two compounds, or groups of compounds, known, respectively, as asphaltene and petrolene. Petrolene is distinguished from asphaltene through the fact that petrolene is soluble in naphtha while asphaltene is not.

The grahamite heretofore mentioned, on the other hand, is soluble only to the extent of about fifteen per cent. of its weight in carbon tetrachlorid, and to the extent of less than one per cent. of its weight in naphtha. It is accordingly substantially devoid of the so-called petrolene constituents of the meltable asphalts, like uintahite, and is also to a large extent unlike the solid or asphaltene constituents of these minerals. By the practice of the process herein described, it has been possible to produce from the mineral grahamite, asphalts which are perfectly meltable without decomposition, wholly soluble in carbon tetrachlorid, and capable of making permanent mixtures in any proportion with the asphaltic fluxes. It therefore follows that the bitumens of which the natural mineral is principally composed are profoundly modified in character.

In carrying out the process a quantity of the selected asphaltite is continuously subjected to heat and pressure for a prolonged period. The desired conditions are conveniently obtained by heating the material in a closed retort as 10, the pressure resulting from the generation and confinement of gas. In the event that a wholly non-melted asphaltite is used, a small proportion of flux is desirably added. If the flux employed contain paraffin hydrocarbons, the gas for providing the pressure comprises methane, supplied by the cracking of the paraffin hydrocarbons, this cracking of the paraffin hydrocarbons also resulting in the formation of a black solid hydrocarbon which becomes associated with the mass and is a constituent of the finished product.

For the purpose of demonstrating that this is so, I have carefully prepared a small

quantity of a pure solid paraffin hydrocarbon shown by combustion analysis to have the formula  $C_{28}H_{58}$ . For this purpose I extracted a commercial paraffin scale having a melting point of 124 degrees Fahrenheit, with a light gasoline and precipitated the paraffin hydrocarbon from this solution with acetic ether, the extraction of the precipitate with a light gasoline and the reprecipitation of the paraffin from the solution being repeated until the crystalline character of the precipitate, observed with a microscope, showed the precipitate to be a pure product. This product was cracked by heat producing a gas and a black solid hydrocarbon soluble in carbon tetrachlorid, but not soluble in naphtha. A combustion analysis of the black solid hydrocarbon showed it to have the composition  $C_{19}H_{22}$ , and a Hempel analysis of the gas showed it to consist principally of methane. It therefore follows that the cracking of the paraffin hydrocarbon  $C_{28}H_{58}$  is substantially represented by the equation—



Furthermore in the commercial practice of the invention I preferably provide the retort 10 with a gas outlet 17 to which a laterally opening pet cock 18 is applied to permit of the removal of samples of the gas. A Hempel analysis of samples of gas drawn from this pet cock shows that the gas consists principally of methane.

The commercial practice of the process does not require the selection of a pure paraffin as the source of the paraffin hydrocarbon. It is suggested that any material capable of being cracked by heat into an inert gas and a residue miscible with the modified bitumens will serve as a flux when any is required. Inasmuch as the resulting product is a meltable asphalt, a mixture of paraffin hydrocarbons and asphalts, as in the residuum from a mixed base petroleum, may be employed. The asphalts occurring in the residuum from the mixed base petroleums are in no wise objectionable, but are simply retained as constituents of the finished product. In treating the grahamite heretofore mentioned, a residuum from mixed base (Illinois) petroleum, of the grade commercially known as 12°-14° Baumé flux oil, has been found to yield satisfactory results. Analysis has shown that this residuum contains from two to four per cent. of solid paraffin.

A continued application of heat and pressure alone suffices for the production of a meltable product. The reaction is expedited, however, and the resulting product greatly improved if a reducing agent be provided as by the liberation of nascent hydrogen in the heated batch. This liberation of nascent hydrogen has been conveniently ac-

complished by the reaction of caustic soda upon iron, in accordance with the equation



For this purpose a quantity of dry caustic soda is used and the treatment is carried on in an iron retort. The caustic soda is thereby permitted to react upon the iron walls of the retort. While this procedure results in an erosion of the iron walls of the retort, the action in this respect has been found to be so slight that the deterioration of the retort is substantially negligible.

A mixture consisting of seventy-four percent. by weight of the grahamite, heretofore mentioned, twenty-four per cent. by weight of the 12° to 14° Baumé flux oil from Illinois petroleum, and one per cent. by weight of dry caustic soda, if held in a closed iron retort and subjected to a temperature of 400° Fahrenheit and a resulting pressure of fifty pounds per square inch for a period of twenty-four hours, produces a lustrous black solid asphalt melting at 380° Fahrenheit, perfectly soluble in carbon bisulfid and carbon tetrachlorid and soluble to the extent of forty-three per cent. of its weight in naphtha.

This product, while having a conoidal fracture and otherwise resembling a natural uintahite (gilsonite), is distinguished therefrom by having a higher melting point and by being pure black in powdered form, but more particularly by containing a larger proportion of constituents soluble in naphtha and by being more viscous when first melted. Preferably the selected quantity of petroleum residuum is first introduced into the retort 10 and heated alone to a temperature of 250° Fahrenheit. The filling opening 11 of the retort may be left open during this part of the process, if desired. The full quantity of grahamite in lump form and the caustic soda is then added and the filling opening 11 sealed with a man-hole cover 12. The heating of the retort is accomplished by the maintenance of a suitable fire in the furnace 13. As shown, this furnace is constructed with return flues 21, 22, one extending along each side of the retort 10. These return flues lead to a stack (not shown), through down-comers 23, 24, and a smoke tunnel 25. Preferably the retort 10, is provided with a pressure gage 14 and with a depending tube 15, closed at its lower end, for the introduction of a thermometer (not shown), to permit observations of the pressure and temperature to be made from time to time. In order that the desired pressure may be attained but not exceeded the gas outlet pipe 17 is provided with an automatic pressure regulating valve 19 which may be adjusted to permit the flow of gas through the pipe only when the desired pressure, as 50 lbs., per square inch, is reached. It is also ad-

visible to provide the retort 10 with safety valves 16, two of which are shown, as a precaution against a dangerous rise in pressure in event the gas is produced with too great rapidity to pass off through the outlet pipe 17. I prefer to adjust the safety valves 16 to open at a pressure which exceeds that at which the pressure regulating valve 19 opens by about two pounds per square inch. The completed product is most conveniently withdrawn from the retort while still soft, as through an outlet pipe 26 controlled by a valve 27. This pipe is preferably protected from direct exposure to the heat of the fire, as by being inclosed with masonry walls 28.

A comparison of the original grahamite and the resulting product, obtained by the use of the process in the specific manner herein described, is conveniently shown by the following table:

|                                           | Grahamite.  | Product.             |
|-------------------------------------------|-------------|----------------------|
| 25 Appearance .....                       | Dull black. | Lustrous black.      |
| Character .....                           | Friable.    | Conchoidal fracture. |
| Specific gravity .....                    | 1.16        | 1.12                 |
| Portion soluble in CS <sub>2</sub> .....  | 97.13%      | 99.37%               |
| Portion soluble in CCl <sub>4</sub> ..... | 14.73%      | 99.25%               |
| Portion soluble in naphtha.....           | 0.87%       | 43.05%               |

30 It will be observed that the portion soluble in naphtha is increased by an amount greater than the entire addition of petroleum residuum, and that a considerable portion of bitumen originally insoluble in 35 carbon tetrachlorid has been so modified as to be completely extracted by this solvent. As a further evidence of the modification of the original constituents it is found that the product is entirely free from paraffin.

40 The character of the resulting product may be varied by the use of different relative proportions of flux and the selected asphaltite, a larger proportion of flux being employed when a product having a lower 45 melting point is desired. Modifications in the character of the product may also be made by varying the temperature, the pressure, or the length of time during which the materials are subjected to treatment. These 50 modifications of the process permit the manufacture of products having melting points which vary from 150° Farhenheit to 420° Fahrenheit. In so far as these products are comparable, as to their melting 55 points, with natural uintahite, the portion of the product soluble in naphtha is in each case greater than in the natural uintahite melting at the same temperature. The temperature to which the mixed materials are 60 subjected is preferably about 20° Fahrenheit above the melting point desired for the finished product, as naphthas of different specific gravity and from different sources behave differently as solvents of asphalt constituents, it is noted that the naphtha herein 65

referred to is of 50° Baumé from Illinois crude petroleum and is used as a solvent at the room temperature.

I claim as my invention—

1. The improved process of treating non-meltable or imperfectly meltable bitumen to render it meltable, which consists in subjecting the same to the simultaneous action of heat and a fluid pressure of substantial intensity above that of the atmosphere and continuing the treatment until a homogeneous melted product is obtained.

2. The improved process of treating non-meltable or imperfectly meltable bitumen to render it meltable, which consists in mixing the same with a quantity of paraffin hydrocarbon and subjecting the mixture to the action of heat in a retort constructed for the confinement of the generated gas at high pressure, and continuing the treatment until a homogeneous melted product is obtained.

3. The improved process of treating non-meltable or imperfectly meltable bitumen to render it meltable, which consists in mixing the same with a quantity of paraffin hydrocarbon and an alkali and exposing the mixture to a metal and to the action of heat in a retort constructed for the confinement of the generated gas at high pressure and continuing the treatment until a homogeneous melted product is obtained.

4. The improved process of treating non-meltable or imperfectly meltable bitumen to render it meltable, which consists in subjecting the same to the simultaneous action of heat and pressure and to that of nascent hydrogen, and continuing the treatment until a homogeneous melted product is obtained.

5. The improved method of manufacturing a meltable asphalt which consists in subjecting a mixture of a mixed base petroleum residuum and an asphaltic coal to the application of heat in a retort constructed for the confinement of the generated gas at high pressure and continuing the treatment until a homogeneous melted product is obtained.

6. The improved method of manufacturing a meltable asphalt which consists in subjecting a mixture of a mixed base petroleum residuum and an asphaltic coal with agents for the production of nascent hydrogen to the application of heat in a retort constructed for the confinement of the generated gas at high pressure, and continuing the treatment until a homogeneous melted product is obtained.

7. The improved method of manufacturing a meltable asphalt which consists in subjecting a mixture of a mixed base petroleum residuum, an asphaltic coal, and an alkali to the application of heat in an iron retort constructed for the confinement of the generated gas at high pressure and continuing

the treatment until a homogeneous melted product is obtained.

8. The improved method of manufacturing a meltable asphalt which consists of the application of heat to a non-meltable bitumen in the presence of gas while the said materials are held in a retort which is constructed for the confinement of the gas at high pressure, and continuing the treatment until a homogeneous melted product is obtained.

9. The improved method of manufacturing a meltable asphalt which consists of the application of heat to a non-meltable bitumen in the presence of an inert gas and agents for the production of nascent hydrogen while the said materials are held in a retort which is constructed for the confinement of the gas at high pressure and continuing the treatment until a homogeneous melted product is obtained.

10. The improved method of treating a non-meltable bitumen to produce meltable asphalt which consists in subjecting the same to the action of heat in the presence of agents which are cracked by heat to produce a gas and a residue which is miscible with the bitumen while the said materials are held in a retort which is constructed for the confinement of the gas at high pressure, and continuing the treatment until a homogeneous melted product is obtained.

11. The improved process of treating non-meltable or imperfectly meltable bitumen to produce a meltable asphalt which consists in subjecting the same to the simultaneous action of heat, pressure and a reducing agent and continuing the treatment until a homogeneous melted product is obtained.

12. The improved method of manufacturing a meltable asphalt which consists of the application of heat to a non-meltable bitumen in the presence of gas and a reducing agent while the said materials are held in a retort which is constructed for the confinement of the gas at high pressure and continuing the treatment until a homogeneous melted product is obtained.

13. The improved method of manufacturing meltable asphalt, which consists of the application of heat to a mixture of a non-meltable bitumen and an agent from which gas is evolved when heated, while the said materials are held in a retort which is constructed for the confinement of the gas at high pressure, and continuing the treatment until a homogeneous melted product is obtained.

14. The improved method of manufacturing meltable asphalt which consists of the application of heat to a material comprising a non-meltable bitumen and from which gas is evolved when heated while the said material is held in a retort which is constructed for the confinement of the gas at high pres-

sure and continuing the treatment until a homogeneous melted product is obtained.

15. The improved method of reducing the amount of paraffin in asphalt containing paraffin which consists in subjecting the said asphalt to the simultaneous action of heat and a fluid pressure of substantial intensity above that of the atmosphere and continuing the treatment until the said paraffin has been cracked to produce asphaltene. 75

16. Prepared meltable asphalt characterized by substantially complete solubility in carbon tetrachlorid and by comprising a greater proportion of petrolene than is found in natural uintalite melting at a temperature which is not higher than the melting point of the said prepared asphalt. 80

17. Prepared asphalt melting at 380 degrees Fahrenheit and comprising asphaltene fifty-six per cent. and petrolene forty-three per cent. 85

18. Prepared asphalt solid at ordinary temperatures but meltable without decomposition, of lustrous black appearance, conchoidal fracture and possessing the characteristics of a product obtained by prolonged exposure of a natural non-meltable asphaltite to heat and pressure. 90

19. Prepared asphalt solid at ordinary temperatures but meltable without decomposition, of lustrous black appearance, conchoidal fracture, and possessing the characteristics of a product obtained by prolonged exposure of a natural non-meltable asphaltite to heat and pressure with agents for the production of nascent hydrogen. 95

20. Prepared asphalt comprising petrolene which petrolene is of a black color and solid at ordinary temperatures. 100

21. Prepared asphalt solid at ordinary temperatures but meltable without decomposition, of lustrous black appearance, conchoidal fracture, and possessing the characteristics of a product obtained by prolonged heating of a mixture of a natural non-meltable asphaltite and petroleum residuum in a closed retort. 105

22. Prepared asphalt solid at ordinary temperatures but meltable without decomposition, of lustrous black appearance, conchoidal fracture, and possessing the characteristics of a product obtained by prolonged heating of a mixture of a natural non-meltable asphaltite, petroleum residuum, and agents for the production of nascent hydrogen in a closed retort. 115

23. Prepared asphalt solid at ordinary temperatures but meltable without decomposition, of lustrous black appearance, conchoidal fracture, and possessing the characteristics of a product obtained by prolonged heating of a mixture of a natural non-meltable asphaltite, petroleum residuum, and an alkali in a closed iron retort. 125

24. Prepared asphalt comprising petro- 130

- lene which petrolene is solid at ordinary temperatures.
25. Prepared asphalt free from paraffin.
26. Prepared asphalt comprising petro-  
5 lene which petrolene is of a black color.
27. Prepared asphalt comprising asphal-  
tene which asphaltene is of a black color,  
solid at ordinary temperatures but melting  
at 228° F. and contains carbon and hydrogen  
10 in proportions represented by the formula  
 $C_{19}H_{22}$ .

28. Prepared asphalt comprising asphaltene which asphaltene is of the character re-  
sulting from the cracking of paraffin by pro-  
longed exposure to heat and a fluid pressure 15  
of substantial intensity above that of the  
atmosphere.

RUDOLPH R. ROSENBAUM.

Witnesses:

CHARLES B. GILLSON,  
E. M. KLATCHER.